# EUROPEAN PATENT SPECIFICATION

(11) **EP 4 249 571 B1**
(45) Date of publication and mention of the grant of the patent: **17.12.2025**
(21) Application number: 21895219.0
(22) Date of filing: 28.05.2021
(51) Int. Cl.: C10B 57/04

(54) **COMPOSITION OF A CHARGE FOR PRODUCING METALLURGICAL COKE**
ZUSAMMENSETZUNG EINER CHARGE ZUR HERSTELLUNG VON METALLURGISCHEM KOKS
COMPOSITION DE CHARGE POUR PRODUIRE DU COKE MÉTALLURGIQUE

(30) Priority: 19.11.2020 RU 2020138082
(43) Date of publication of application: 27.09.2023
(73) Proprietor: NLMK International B.V., 1077 XX Amsterdam (NL)
(72) Inventor: PRUS, Andrei Andreevich, Moscow, 117638 (RU); TIMIN, Evgeny Nikolaevich, Moscow, 108811 (RU); DENISENKO, Elena Viktorovna, Altai Kray, 659100 (RU); VIUKOV, Dmitrii Sergeevich, Lipetsk, 398046 (RU); KAPUSTIN, Vladimir Mikhailovich, Moscow, 119296 (RU)
(74) Representative: Boskovic, Davor
(86) International application number: PCT/RU2021/050148
(87) International publication number: WO 2022/108484

(56) References cited:
- EP-A1- 2 103 667
- EA-B1- 021 524
- RU-C1- 2 174 528
- RU-C1- 2 627 425
- RU-C1- 2 637 699
- SU-A1- 1 736 993
- "GOST 25543-2013; Brown coals, hard coals and anthracites CLASSIFICATION ACCORDING TO GENETIC AND TECHNOLOGICAL PARAMETERS", INTERSTATE STANDARD, 2014, Moscow
- " Ugolnyye i grafitovyye konstruktsionnyye materialy [Carbon and graphite structural materials]", vol. 226, 30 November 1965, IZDATELSTVO 'NAUKA, Moscow, article VESELOVSKII V. S: "Deystviye otoshchayushchikh dobavok] Action of lean supplements", pages: 121 - 124, XP009537345

## Description

The invention relates to the coke industry and in particular to the composition of a charge for producing metallurgical coke.

It is known that in order to improve the technological characteristics of charges, to upgrade the quality of coke, and to save scarce coal ranks, it is proposed to use various organic additives, such as solid waste from coke production, petroleum coke breeze, non-caking coals, and other additives, while ensuring the strength characteristics of coke and reducing the cost of production.

There is a known charge used for metallurgical coke comprising a coking coal, a coke production waste plasticizer in the amount from of 0.5 to 7 wt.% (RU No. 2333236, 10.09.2008), and bituminous residue from the process of producing light fractions of petroleum products, and having the following characteristics: ash content A^{d} is up to 2.5%; volatiles content V^{daf} is up to 70%; sulfur content S^{d} is up to 5%; swelling is not less than 20 mm; and Roga index (RI) is not less than 10 (RU No. 2418837, 20.05.2011).

A significant disadvantage of using the above inventions is the impossibility of using plastic components in the charge of coke production due to possible agglomeration of particles and sticking, the need to reconstruct technological equipment in a coal preparation or coke departments, as well as the possibility of replacing only certain ranks of coking coal due to a relatively low level of volatile substances.

There is a known method (RU No. 2663145, 01.08.2018) of producing a charge for coking, which comprises mixing a petroleum caking additive with low-caking coal ranks CC (coking low-caking) and/or CLCLM (coking low-caking low-metamorphosed coals), and/or CL (coking lean), and/or LL (lean low-caking) and/or LC (lean caking) in the following ratio of components, wt.%:
- petroleum caking additive - from 1 to 30,
- low-caking coals - from 99 to 70.

The petroleum caking additive is a petroleum refining residue having the following characteristics:
- ash content A^{d} - up to 2.5%;
- volatiles content V^{daf} - up to 90%;
- sulfur content S^{d} - up to 5%;
- ring-and-ball softening point - not less than 40°C.

The disadvantage of this invention is the lack of technologies for supplying components in a liquid-flow state to the coal charge and, as a result, the impossibility of applying the invention in an industrial scale.

There is a known charge composition used for coking and comprising a petroleum additive being the product of delayed semi-coking of heavy petroleum residues with a volatile content of 12 to 28 wt.%. (RU No. 2355729, 20.05.2009; No. 2411283, 10.02.2011; RU No. 2563493, 2015; RU No. 2637965, 08.12.2017).

The disadvantage of the additive according to these patents is the instability of its caking properties, the insufficient coking level of the additive and, accordingly, the unstable quality of the resulting metallurgical coke, as well as the lack of a description of clear boundaries for the use of this product in the composition of the charge for coke production, which causes difficulties in assessing the effect of the presence of this product on the quality of metallurgical coke.

Further, there is a known blend of petroleum coke used in the charge composition in the amount of 1-30 wt.%. and petroleum residues in the amount of 1-30 wt%.

The used petroleum residues are characterized by ash content A^{d} of up to 2.5%, volatiles content V^{daf} of up to90%, sulfur content S^{d} of up to5%, and Roga index (RI) of less than 10. The petroleum coke is characterized by ash content A^{d} of up to2.5%, volatiles content V^{daf} of up to25%, and sulfur content S^{d} up to5% (RU No. 2627425, 08.08.2017).

A significant disadvantage of using the invention is the need to reconstruct the process equipment in the coal preparation or coke departments.

Patent document RU 2 174 528 C1, 10.10.2001, discloses a method for producing coke from a charge containing a mixture of:
60% of coals of caking groups: GF (gas fat coal) and/or F (fat coal);
25% of coking coals;
0-15% of coals of inert groups of ranks CC (coking low-caking coal) and/or LC (lean caking coal) and/or lean coking coal;
0-15% of petroleum coke fines.

The disadvantage of the described method is high consumption of valuable caking and coking coals and low consumption of coals of inert groups with achievement of not sufficiently favorable parameters: quite low CSR (coke strength after reaction with CO₂ (%)) and high CRI (coke reactivity index (%)).

The closest composition of the charge for coking is the composition of the charge proposed in the method for producing metallurgical coke (RU No. 2553116, 2015), which is used as a carbonaceous charge with a content of from 50 to 100 wt.% of petroleum semi-coke with a volatiles content of from 14 to 25 wt.% produced by delayed partial carbonization of heavy petroleum residues.

The disadvantage of the described method using a carbonaceous charge is the difficult use of the equipment made specifically for this method.

The problem to be solved by the invention is to develop a special coking charge composition, which makes it possible to expand the range and reduce the cost of the raw materials of the used charge with an improvement in the quality of metallurgical coke having higher strength characteristics (coke strength after reaction with CO₂ (CSR) in the range of from 60 to 66% and coke reactivity index (CRI) in the range of form 23 to 28%).

This problem is solved by developing a special coking charge composition for producing metallurgical coke, comprising:
- a blend of coals of caking groups: ranks G (gas coal) and/or GF (gas fat coal) and/or GFL (gas fat lean coal) and/or F (fat coal), and inert groups of ranks CC (coking low-caking coal) and/or LC (lean caking coal) in a mass ratio of 1:1.15 (a blend of coals of caking groups comprises coals of ranks G, GF, GFL, F, as well as coals of LC and CC ranks within the blends of inert groups , respectively, can be used as interchangeable without deterioration of characteristics of the resulting coke),
- a petroleum coke produced by the delayed coking of heavy petroleum residues, which has a caking index of from 75 to 100 units (GOST ISO 15585-2013), with the following ratio of components, wt.%:
   blend of coals of caking and inert groups in a mass ratio of 1:1.15 - 60 to 93.5; and
   petroleum coke - 6.5 to 40.

The charge composition uses petroleum coke produced by delayed coking of heavy petroleum residues: tar, deasphalting asphalt, vacuum visbreaking residue, etc.

The experiments conducted by the authors of the present invention with charges of various rank composition at a mass ratio of coals of caking and inert groups of 1:1.15 with petroleum coke added to the blend in an amount of from 6.5 to 40 wt.% showed that it is possible to produce metallurgical coke having improved strength characteristics.

The possibility of replacing the coal component with petroleum coke is explained by the fact that petroleum coke has a dual effect on the caking process: it acts on the one hand as a lean additive, and on the other hand, as a caking component, since petroleum coke comprises liquid products and can affect the pyrolysis processes of carbon mass.

### Exemplary embodiments

### Example 1

For the implementation of the invention, the used charge for the coke production had the following composition, wt.%: $\left(G+GF+GFL+F\right) = 43.5 wt . % ;$ CC = 50.0 wt.%; petroleum coke = 6.5 wt.% $\left(G+GF+GFL+F\right) : \left(CC\right) = 1 - 1.15 ;$

Table 1 represents the qualitative characteristics of petroleum coke.

**Table 1**

| | Parameter | Unit | Value |
|---|---|---|---|
| 1 | Ash content A^{d} | % | 0.4 |
| 2 | Volatiles content V^{d} | % | 15-18 |
| 3 | Total sulfur content S^{d} | % | 4.0-4.8 |
| 4 | Coke strength after reaction CSR | % | 55-70 |
| 6 | Coke reactivity index CRI | % | 23-28 |
| 7 | Caking index G, GOST ISO 15585-2013 | - | 75-100 |

Similarly, for the implementation of the invention, the used charge according to examples 2 and 3 had a ratio of caking and inert coal groups of 1:1.15. Table 2 represents the qualitative characteristics of metallurgical coke depending on the charge composition and the amount of petroleum coke used.

**Table 2**

| Charge version | Charge composition, % | | | Physical and chemical properties of metallurgical coke, % | | | | |
|---|---|---|---|---|---|---|---|---|
| | G + GF + GFL + F | CC/LC | Petroleum coke | W^{r} | A^{d} | S^{d} | CSR | CRI |
| Basic | 46.5 | 53.5 | 0 | 0.2 | 11.1 | 0.52 | 57.2 | 30.0 |
| Experimental 1 | 43.5 | 50.0 | 6.5 | 0.2 | 10.4 | 0.75 | 60.4 | 28.0 |
| Experimental 2 | 38.6 | 44.4 | 17.0 | 0.2 | 9.3 | 1.15 | 63.8 | 24.3 |
| Experimental 3 | 27.9 | 32.1 | 40.0 | 0.2 | 6.9 | 1.85 | 65.8 | 23.1 |

where W^{r} is total moisture content (%); A^{d} is ash content (%); S^{d} is total sulfur content (%); CSR is coke strength after reaction with CO₂ (%); and CRI is coke reactivity index (%).

As follows from the data given in Table 2, charges comprising blends of caking and inert coal groups of various ranks in the ratio of 1: 1.15 in the amount of from 60 to 93.5 wt.% and petroleum coke in the amount of from 6.5 to 40 wt.% can be used to produce metallurgical coke with improved strength characteristics: coke strength after reaction with CO₂ (CSR) in the range of from 60 to 66% (57% in the basic version) and coke reactivity (CRI) in the range of from 23 to 28% (30% in the basic version).

## Claims

1. A charge of a special composition for the production of metallurgical coke, comprising
- a blend of coals of caking groups: ranks gas coal and/or gas fat coal and/or gas fat lean coal and/or fat coal, and inert groups: ranks coking low-caking coal and/or lean caking coal, in a mass ratio of 1:1.15; and
- a petroleum coke produced by the delayed coking of heavy petroleum residues, which has a caking index of from 75 to 100 units (GOST ISO 15585-2013),
with the following ratio of components, wt.%:
blend of coals of caking and inert groups in a mass ratio of 1:1.15 - 60 to 93.5; and
petroleum coke - 6.5 to 40.

## Patentansprüche

1. Eine Charge einer besonderen Zusammensetzung zur Herstellung von Hüttenkoks, bestehend aus
- einer Mischung aus Kohlen der verbackenden Gruppen: Ränge Gaskohle und/oder gasförmige Fettkohle und/oder gasförmige magere Fettkohle und/oder Fettkohle und inerte Gruppen: Ränge verkokende, leicht verbackende Kohle und/oder magere verbackende Kohle, in einem Massenverhältnis von 1:1,15; und
- dem Petrolkoks, der durch verzögerte Verkokung schwerer Erdölrückstände hergestellt wird und einen Verbackungsindex von 75 bis 100 Einheiten (GOST ISO 15585-2013) hat,
mit dem folgenden Verhältnis der Komponenten, Gew. %:
Mischung aus Kohlen aus verbackenden und inerten Gruppen im Massenverhältnis 1:1,15 - 60 bis 93,5; und Petrolkoks - 6,5 bis 40.

## Revendications

1. Charge d'une composition spéciale pour la production de coke métallurgique, comprenant
- un mélange de charbons de groupes agglomérants : rangs de charbon gazeux et/ou charbon gras gazeux et/ou charbon gras gazeux maigre et/ou charbon gras, et de groupes inertes : rangs de charbon cokéfiant faiblement agglomérant et/ou charbon maigre agglomérant, dans un rapport massique de 1:1.15; et
- un coke de pétrole issu de la cokéfaction retardée de résidus pétroliers lourds, qui présente un indice d'agglomération de 75 à 100 unités (GOST ISO 15585-2013),
avec le rapport de composants suivant, % en poids :
mélange de charbons agglomérants et de groupes inertes dans un rapport massique de 1:1.15 - 60 à 93.5; et coke de pétrole - 6,5 à 40.
